

April 28, 1964

S. ILNYKYJ ET AL  
PROCESS FOR THE MANUFACTURE OF POUR DEPRESSANTS  
FOR MIDDLE DISTILLATE FUELS  
Filed Jan. 5, 1960

3,131,168



Stephan Ilnykyj  
John L. Tiedje  
By *W. O. Helmman*  
Inventors  
Patent Attorney

## 1

3,131,168

## PROCESS FOR THE MANUFACTURE OF POUR DEPRESSANTS FOR MIDDLE DISTILLATE FUELS

Stephan Incykyj and John L. Tiedje, Sarnia, Ontario, Canada, assignors to Esso Research and Engineering Company, a corporation of Delaware

Filed Jan. 5, 1960, Ser. No. 593  
1 Claim. (Cl. 260—87.3)

The present invention is concerned with the manufacture of improved pour depressants, particularly, for use with middle distillates. The pour depressant of the present invention comprises copolymers of ethylene with up to about 50% by weight of an olefinically unsaturated aliphatic monomer containing from about 3 to 5 carbon atoms per molecule. The copolymers of a particular average molecular weight are obtained by controlling the conditions of reaction. The preferred copolymer of the present invention is a particular copolymer of ethylene and vinyl acetate and is particularly directed toward the method of manufacture wherein reagents are continuously added.

With the increase in the use of hydrocarbon fuels of all kinds, a serious problem has arisen in areas frequently subjected to low temperatures in the cold test characteristics of fuels. Particularly, serious problems have been encountered with heating oils and diesel and jet fuels that have too high a pour point, resulting either in distributional or operating difficulties or both. For example, the distribution of heating oils by pumping or siphoning is rendered difficult or impossible at temperatures around or below the pour point of the oil. Furthermore, the flow of the oil at such temperatures through the filters cannot be maintained, leading to the failure of the equipment to operate.

Also the low temperature properties of petroleum distillate fuels boiling in the range between about 250° and about 750° F. have attracted increasing attention in recent years because of the growth of market for such fuels in subarctic areas and because of the development of turbo-jet aircraft capable of operating at altitudes where temperatures of —50° F. or lower may be encountered.

It is, therefore, an object of the present invention to set forth an improved process for the manufacture of very effective pour depressants for middle distillates and lighter oils. In general, these oils boil in the range from about 250° to 750° F.

It is a still further object of the present invention to provide heating oils, diesel fuel oils, kerosines and jet fuels having low pour points. Aviation turbo-jet fuels in which the polymers may be used normally boil between about 250° and about 550° F. and are used in both military and civilian aircraft. Such fuels are more fully defined by U.S. Military Specifications MIL-F-5624C, MIL-F-25554A, MIL-F-25558A, and amendments thereto. Kerosines and heating oils will normally have boiling ranges between about 300° and about 750° F. and are more fully described in ASTM Specification D-396-48T and supplements thereto, where they are referred to as No. 1 and No. 2 fuel oils. Diesel fuels in which the polymers may be employed are described in detail in ASTM Specification D-975-53T and later versions of the same specification.

The process of the present invention produces copoly-

## 2

mers of ethylene and up to about 50% by weight of an olefinically unsaturated aliphatic monomer containing from about 3 to 5 carbon atoms per molecule. In general, these compounds may comprise vinyl acetate, vinyl propionate, methyl methacrylate, allyl ethyl ether, divinyl ether, acrylonitrile, vinylacetonitrile and the like.

The preferred copolymers comprise ethylene-vinyl acetate copolymer. It is preferred that the parts by weight of ethylene in the copolymer be in the range from about 60 to 99% as compared to parts by weight of vinyl acetate in the range from about 40 to about 1%. A very desirable polyethylene vinyl acetate copolymer contains about 15 to 28% by weight of vinyl acetate, as for example, about 20 parts by weight of vinyl acetate.

The molecular weights of the ethylene-vinyl acetate copolymer are critical and should be in the range from about 1,000 to 3,000, preferably, in the range from about 1,500 to 2,200. The molecular weights are determined by K. Rast's method (Ber. 55, 1051, 3727 (1922)).

The ethylene-vinyl acetate copolymer as described above is used in a concentration in the range from about .001 to 0.2% by weight, preferably, in a concentration in the range from about .005 to .1% by weight.

In accordance with the present invention, the polymerization process is conducted in a solvent as, for example, toluene or hexane. It is preferred, however, to use a benzene solvent. The initiator comprises any peroxy compound, preferably, di-tertiary-butyl-peroxide. The temperature of the polymerization reaction is in the range from about 280° to 340° F. A very desirable temperature is about 300° F. The pressure is in the range from about 700 to 2,000 pounds, preferably, 800 or 900 pounds. The autoclave or similar equipment containing the solvent, initiator and vinyl acetate is purged with nitrogen, then with ethylene before charging with a sufficient amount of ethylene to yield the desired pressure when heated to the reaction temperature. During the polymerization, additional ethylene is added to maintain the pressure at the desired level. Polymerization is considered complete when the pressure drops less than 50 p.s.i.g. per hour. The product is stripped free of solvent and unreacted vinyl acetate under vacuum.

In accordance with the present invention, the reagents are continuously added. A number of operations were carried out in order to establish the optimum conditions for the manufacture of the pour depressant of the present invention.

In other operations, reactants were continuously fed to the reactor. In the first phase of this operation, vinyl acetate was charged into the reactor at the start of each run and di-tertiary-butyl-peroxide in 25% concentration in benzene was fed continuously as the copolymerization proceeded. Table I compares products obtained with the best copolymer, A, produced when all reactants were charged to the reactor at the beginning of the reaction.

The effect of reaction variables on yield and potency of pour depressant was studied in some detail. Generally it was found that the yield of copolymer increased with polymerization time, slower rate of addition of initiator, and increases in pressure. In the range studied, the highest potency pour depressant was obtained when operating at 650 p.s.i.g. and using short polymerization times with fast addition of peroxide. When considering both yield and quality of pour depressant, the best product was obtained at 900 p.s.i.g., 300° F., 3 hours' total polymerization time and 1 hour addition time of peroxide.

TABLE I  
*Pilot Copolymerization of Ethylene and Vinyl Acetate*  
[All vinyl acetate charged at start, continuous addition of peroxide]

| Operation                       | A    | B    | C    | D     | E    | F    | G     | H     | I    |
|---------------------------------|------|------|------|-------|------|------|-------|-------|------|
| Reactor Conditions:             | 12   | (2)  | (2)  | (2)   | (2)  | (2)  | (2)   | (2)   | (2)  |
| Vinyl acetate, ml.              | 30   | 150  | 150  | 150   | 150  | 120  | 120   | 120   | 90   |
| Peroxide, ml.                   | 5    | 15   | 15   | 15    | 15   | 15   | 15    | 15    | 15   |
| Peroxide addition, hrs.         | 0    | 4    | 1    | 1     | 1    | 1    | 1     | 1     | 1    |
| Polymerization, hrs.            | 6    | 6    | 6    | 3     | 3    | 3    | 6     | 6     | 6    |
| Pressure, p.s.i.g.              | 850  | 900  | 900  | 1,200 | 900  | 650  | 650   | 650   | 550  |
| Temperature, °F.                | 300  | 300  | 300  | 300   | 300  | 300  | 300   | 280   | 300  |
| Product:                        |      |      |      |       |      |      |       |       |      |
| Yield, g.                       | 100  | 731  | 615  | 585   | 530  | 414  | 434   | 396   | 352  |
| Initiator efficiency            | 25   | 61.4 | 51.7 | 49.2  | 44.5 | 34.8 | 36.5  | 33.3  | 29.5 |
| Vinyl acetate, wt. percent.     |      |      |      |       |      |      |       |       |      |
| Pour depressant, °F.:           | 20.4 | 15.8 | 20.6 | 18.8  | 21.9 | 22.8 | 21.0  | 21.9  | 20.9 |
| 0.05 wt. percent.               | 60   | 25   | 50   | 40    | 60   | 65   | 50    | 75    | 15   |
| 0.1 wt. percent.                | >90  | 40   | 80   | 65    | 80   | >100 | 90    | >90   | 80   |
| Vinyl Acetate Balance:          |      |      |      |       |      |      |       |       |      |
| Polymerized, wt. percent.       | 72.9 | 87.5 | 90.6 | 78.7  | 83.0 | 84.4 | 81.3  | 77.5  | 87.4 |
| Recovered monomer, wt. percent. |      |      |      |       |      |      |       |       |      |
| Unaccounted for, wt. percent.   | 4.9  | 8.2  | 7.9  | 13.3  | 11.3 | 4.7  | ----- | 7.6   |      |
|                                 | 27.1 | 7.6  | 1.2  | 13.4  | 3.7  | 4.2  | 14.0  | ----- | 5.0  |

<sup>1</sup> Litres. <sup>2</sup> One gallon. <sup>3</sup> Av.

Further improvements in the process were obtained when the vinyl acetate was continuously added to the reactor as the polymerization reaction proceeded. These runs are shown in Table II.

In general, the manufacture of the copolymer of the present invention is carried out at a temperature in the range from about 280° to 340° F., preferably at about 300° F. The pressure is in the range from about 700 to

TABLE II

*Pilot Copolymerization of Ethylene and Vinyl Acetate*

[One gallon reactor, continuous addition of vinyl acetate and peroxide, 900 p.s.i.g., 300° F.]

| Operation                         | A     | B    | C <sup>1</sup> | D <sup>2</sup> | E <sup>2</sup> | F <sup>2</sup> | G     | H <sup>3</sup> |
|-----------------------------------|-------|------|----------------|----------------|----------------|----------------|-------|----------------|
| Conditions:                       |       |      |                |                |                |                |       |                |
| Benzene, ml.                      | 1,395 | 315  | 330            | 1,395          | 345            | 405            | 1,290 | 7,740          |
| Vinyl acetate, total ml.          | 150   | 150  | 150            | 150            | 150            | 150            | 300   | 1,800          |
| Vinyl acetate, at start, ml.      | 150   | 30   | 15             | 150            | 0              | 0              | 0     | 0              |
| Vinyl acetate, balance ml./min.   |       | 0    | 2.0            | 1.1            | 0              | 2.5            | 2.5   | 5              |
| Di-t-butylperoxide, tot. ml.      | 0.15  | 15   | 15             | 15             | 15             | 15             | 15    | 15             |
| Di-t-butylperoxide, ml./min.      | 0.25  | 0.25 | 0.25           | 0.25           | 0.25           | 0.125          | 0.25  | 1.0            |
| Polymerization time, hrs.         | 3     | 3    | 6              | 3              | 3              | 3              | 3     | 3.5            |
| Product:                          |       |      |                |                |                |                |       |                |
| Yield, g.                         | 530   | 343  | 344            | 477            | 314            | 345            | 810   | 6,700          |
| Yield, g./g. peroxide             | 44.5  | 28.9 | 28.9           | 40.0           | 26.3           | 29.0           | 34.0  | 46.9           |
| Vinyl acetate, wt. percent.       | 21.9  | 34.0 | 33.5           | 22.7           | 27.6           | 31.1           | 29.8  | 23.5           |
| Pour depressant, °F. <sup>4</sup> |       |      |                |                |                |                |       |                |
| 0.05 wt. percent.                 | 60    | 55   | 45             | 50             | 35             | 75             | >80   | >90            |
| 0.1 wt. percent.                  | 80    | >85  | 70             | >90            | 90             | 90             | >80   | >90            |
| Vinyl acetate balance:            |       |      |                |                |                |                |       |                |
| Polymerized, wt. percent.         | 83.6  | 83.4 | 82.4           | 77.4           | 77.4           | 77.1           | 86.2  | 93.9           |
| Recovered monomer, wt. percent.   |       |      |                |                |                |                |       |                |
| Unaccounted for, wt. percent.     | 13.3  | 6.0  | 8.2            | 11.4           | 12.4           | 11.3           | 10.5  | -----          |
|                                   | 3.7   | 10.6 | 9.4            | 11.2           | 10.2           | 11.6           | 3.3   | 6.1            |

<sup>1</sup> 800 p.s.i.g.

<sup>2</sup> Inhibitor removed from vinyl acetate.

<sup>3</sup> 5 U.S. gallons reactor.

<sup>4</sup> 50/50 blend of virgin and cat. cracked gas oils, pour +20° F.

The advantages of these operations were improved quality of pour depressant and substantially reduced solvent requirement. This latter factor resulted not only in a reduction of solvent required, but also in much higher utilization of reactor volume. See Table III.

2,000 pounds for a time period of from 2 to 16 hours. The preferred pressure is in the range from about 800 to 1,000, preferably, about 900 pounds. The preferred time of reaction is from about 2 to 6 hours. The concentration of the vinyl acetate in the benzene solution varies from 0.53 to 10%.

A typical preferred method for conducting a polymerization of the present invention is illustrated in the figure. Referring specifically to the figure, reactor 20 is first purged with nitrogen, introduced by means of line 12 and pump 13. Reactor 20 is then purged with ethylene which is introduced by means of line 12 and pump 13. Gases are removed from reactor 20 by means of line 11. The reactor is maintained at a positive pressure in the range from about 50 to 100 pounds absolute.

Approximately 220 parts by weight of benzene is introduced into reactor 20 from benzene storage 1 by means of line 6 and pump 5. Reactor 20 is then raised to a temperature of 300° F. by means of heating element 14 wherein a heating fluid or equivalent is introduced by

TABLE III

*Synthesis of Pour Depressants*

| Conditions:                            | At start | At start   | Continuous |  |
|----------------------------------------|----------|------------|------------|--|
| Vinyl acetate addition                 | do       | Continuous | Do.        |  |
| Di-t-butylperoxide addition            |          |            |            |  |
| Product:                               |          |            |            |  |
| Yield, g./USG reactor space            | 342      | 530        | 1,340      |  |
| Yield, g./g. peroxide                  | 23       | 44.5       | 46.9       |  |
| Benzene, g./g. polymer                 | 5        | 2.3        | 1          |  |
| Vinyl acetate polymerized, wt. percent | 66       | 83         | 94         |  |
| Pour depressant, °F. 10.05 wt. percent | 60       | 60         | 90         |  |

<sup>1</sup> 50/50 blend of virgin gas oil and cat. cracked gas oil, ASTM pour +20° F.

means of line 15 and withdrawn by means of line 16. Reactor 20 is held at 300° F. during the course of the reaction by the removal of heat or by the addition of heat thereto. Ethylene is introduced by means of line 12 so as to raise the pressure of the reactor to about 900 pounds.

The addition of vinyl acetate and of di-tertiary-butyl-peroxide is started concurrently. The vinyl acetate is withdrawn from storage zone 3 and introduced into the reactor by means of line 10 and pump 9. Approximately 55 parts by weight of vinyl acetate is added over a two hour period. The peroxide is introduced by passing benzene into storage zone 2 by means of line 4 and then introducing the solution into the reactor 20 by means of line 8 and pump 7. Approximately 5.5 parts by weight of peroxide are combined with 16.5 parts by weight of benzene. The resulting 22 parts by weight of 25% peroxide solution in benzene is added to reactor 20 over a three hour period.

After the addition of the peroxide has been completed, the reactor is held for an additional one-half hour at a temperature of about 300° F. The ethylene is added continuously so as to maintain the pressure at about 900 pounds. In operation, approximately 934 parts by weight of vinyl acetate are used in conjunction with from about 2,800 to 3,800 parts by weight of ethylene.

At the end of the reaction, the reactor is allowed to cool to about 160° F. and the reaction product is then withdrawn by means of line 17 and passed into separation zone 18. Excess ethylene is removed overhead from separation zone 18 by means of line 19. The polymer product comprising the copolymer in a benzene solution may be withdrawn by means of line 22 and further handled as desired. Under certain instances, it may be desirable to separate at least a portion of the benzene from the copolymer. Under these conditions, the benzene copolymer product is passed to separation zone 30 by means of line 21. Benzene is removed overhead by means of line 24, while a copolymer product is withdrawn by means of line 23.

The quantity mentioned above may be somewhat varied. For example, based upon 55 parts by weight of vinyl acetate, the amount of benzene utilized may vary from

about 180 to 300 parts by weight, and the amount of di-tertiary-butyl-peroxide may vary from about 3 to 8 parts by weight. Also as mentioned, the amount of ethylene utilized varies from about 2,800 to 3,800 parts by weight, or approximately 938 parts by weight of vinyl acetate. The time of reaction also may be varied from about 2 to 4 hours, depending upon other operating variables.

While the above operation has been described utilizing a single reactor, it is to be understood that a plurality of reactors may be employed in a similar manner in order to secure continuous production of the copolymer.

What is claimed is:

Process for the manufacture of a pour depressant consisting essentially of a copolymer of ethylene and vinyl acetate, which copolymer has a molecular weight in the range from about 1500 to 2200 as determined by Rast's method, and is characterized by containing from about 15 to 28% by weight of vinyl acetate which comprises purging a reaction zone with nitrogen and thereafter introducing about 220 parts by weight of benzene into a reaction zone, heating the benzene to a temperature of about 300° F., thereafter pressuring said reaction zone with ethylene to about 900 pounds, thereafter continuously adding about 55 parts by weight of vinyl acetate over a reaction time period of about two hours and also continuously adding over a reaction time period of about three hours about 22 parts by weight of a benzene solution containing about 25% by weight of di-tertiary-butyl-peroxide while maintaining said reaction zone at the conditions specified to produce said copolymer, whereby about 310 parts by weight to 142 parts by weight of ethylene will react with said 55 parts by weight of vinyl acetate.

References Cited in the file of this patent

UNITED STATES PATENTS

|           |              |               |
|-----------|--------------|---------------|
| 2,396,785 | Hanford      | Mar. 19, 1946 |
| 2,414,311 | Larson       | Jan. 14, 1947 |
| 2,450,451 | Schmerling   | Oct. 5, 1948  |
| 2,551,643 | Seger et al. | May 8, 1951   |

FOREIGN PATENTS

|         |        |                |
|---------|--------|----------------|
| 459,662 | Canada | Sept. 13, 1949 |
|---------|--------|----------------|